# EUROPEAN PATENT SPECIFICATION

(11) **EP 0 281 146 B1**
(45) Date of publication and mention of the grant of the patent: **07.08.1991**
(21) Application number: 88103347.6
(22) Date of filing: 04.03.1988
(51) Int. Cl.: G03C 1/30

(54) **Method and composition for hardening gelatin**
Verfahren und Zusammensetzung zum Härten von Gelatine
Méthode et composition pour durcir la gélatine

(30) Priority: 05.03.1987 US 22192
(43) Date of publication of application: 07.09.1988
(73) Proprietor: EASTMAN KODAK COMPANY, Rochester, New York 14650-2201 (US)
(72) Inventor: Chen, Chung Yuan c/o EASTMAN KODAK COMPANY, Rochester New York 14650 (US); Riecke, Edgar Erick c/o EASTMAN KODAK COMPANY, Rochester New York 14650 (US); Harbison, Kenneth George c/o EASTMAN KODAK COMPANY, Rochester New York 14650 (US)
(74) Representative: Brandes, Jürgen, Dr. rer. nat.

(56) References cited:
- TETRAHEDRON LETTERS, vol. 24, no. 36, 1983, pages 3919-3920, Pergamon Press Ltd., London, GB; T. GRAMSTAD et al.: "The reaction of trifluoromethanesulphonic anhydride with carbonyl compounds"
- JOURNAL OF THE AMERICAN CHEMICAL SOCIETY, vol. 102, 1980, pages 6361-6362, American Chemical Society, Columbus, Ohio, US; P.J. STANG et al.: "Preparation and characterization of novel dication ether salts: Ar+OAr+.2CF3SO3-"

## Description

This invention relates to a method and hardener composition for hardening gelatin, particularly in photographic elements.

Gelatin is commonly used as a vehicle in photographic materials. Quite often, numerous layers in photographic elements, such as light-sensitive silver halide layers, filter layers, backing layers, antihalation layers, and overcoat layers, use gelatin as the primary binder.

Photographic elements are generally processed in aqueous processing solutions. Such processing results in excessive swelling and loss of strength of the gelatin binder unless the gelatin has been hardened. If the processing solution is maintained at a warm temperature, e.g., 40°C, the gelatin binder can dissolve, causing the layers of the element to disintegrate, unless the gelatin has been hardened.

A number of compounds have been used to harden gelatin. These include formaldehyde and free aldehydes as described in U.S. Patent 3,232,764, active esters as described in U.S. Patent 3,542,558, epoxy compounds as described in U.S. Patent 3,047,394, aziridines as described in U.S. Patent 2,950,197, and others well-known in the art. These compounds harden, or crosslink, gelatin, thus increasing its mechanical strength and reducing the swellability and solubility of the gelatin in aqueous processing solutions.

The above-described hardening compounds are, however, subject to a number of disadvantages. Some take an exceedingly long time after being cast and dried to give the desired degree of gelatin hardening, requiring elements containing gelatin hardened with those compounds to be aged for an extended time while the hardening process is completed. In other words, these hardeners exhibit after-hardening. Additionally, a number of compounds exhibit adverse effects on the photographic properties of elements in which they are used. Such adverse effects can include an increase in fog or a reduction in light sensitivity or photographic speed.

In order to avoid the time and expense of keeping large quantities of gelatin-containing photographic elements for long periods while the hardening process is completed, a number of so-called fast-acting hardeners have been described in the art. For example, U.S. Patent 4,063,952 describes a carbamoyl pyridinium hardening compound in which the pyridine ring carries a sulfoalkyl substituent. European Patent Application 162,308 describes a chloroformamidinium hardener, and U.S. Patent 4,612,280 describes an N-succinimidyloxyformamidinium hardener. These hardeners, however, suffer from a number of problems. Some of these hardeners exhibit after-hardening. Others have severe handling difficulties due to their hygroscopic nature, or poor hydrolytic stability, or both. Also, some of these hardeners adversely affect either the physical properties of photographic elements in which they are used (e.g., tackiness), or their sensitometric properties (e.g., speed loss). These problems are often aggravated by the fact that relatively large amounts of hardener are often required to achieve the desired hardening effect, leading to relatively large amounts of sometimes deleterious by-products.

It is therefore desirable to provide a hardener that provides rapid and efficient hardening of gelatin, while avoiding adverse side-effects, such as after-hardening.

The present invention provides for hardening of gelatin by combining it with a compound of the formula:

In this formula, R₁ represents hydrogen, substituted or unsubstituted alkyl of 1 to 20 carbon atoms, substituted or unsubstituted aralkyl of 7 to 20 carbon atoms, substituted or unsubstituted aryl of 6 to 20 carbon atoms, substituted or unsubstituted alkenyl, of 2 to 20 carbon atoms, -YR₇,
with Y representing sulfur or oxygen, and R₇, R₈, R₉, R₁₀, and R₁₁ each independently representing substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms. Alternatively, R₈ and R₉, or R₁₀ and R₁₁_{,} may together form a substituted or unsubstituted ring structure. R₁₀ and R₁₁_{,} may each also represent hydrogen. Also, R₁ together with R₂ may form a substituted or unsubstituted heterocyclic ring.

R₂ and R₃ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms, or, combined with R₁ or each other, forms a substituted or unsubstituted hererocyclic ring.

R₄, R₅, and R₆ are defined as are R₁, R₂, and R₃, respectively, and are the same as or different from R₁, R₂, or R₃.

X^{⊖} represents an anion or an anionic portion of the compound to form an intramolecular salt.

Compounds of the invention according to formula (I) are described in further detail below.

R₁ represents hydrogen, substituted or unsubstituted alkyl of 1 to 20 carbon atoms, substituted or unsubstituted aralkyl or 7 to 20 carbon atoms, substituted or unsubstituted aryl of 6 to 20 carbon atoms, substituted or unsubstituted alkenyl of 2 to 20 carbon atoms, -YR₇,
with Y representing sulfur or oxygen, and R₇ R₈, R₉, R₁₀, and R₁₁ each independently representing substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl or 2 to 20 carbon atoms. Alternatively, R₈ and R₉, or R₁₀ and R₁₁ may together form a substituted or unsubstituted ring structure. R₁₀ and R₁₁ may each also represent hydrogen. Also, R₁ together with R₂ may form a substituted or unsubstituted heterocyclic ring, which may be further condensed with another ring.

Examples of R₁ include hydrogen, substituted or unsubstituted alkyl of 1 to 20 carbon atoms (e.g., methyl, ethyl, butyl, 2-ethylhexyl, or dodecyl), substituted or unsubstituted aralkyl of from 7 to 20 carbon atoms (e.g. benzyl, phenethyl), substituted or unsubstituted aryl of from 6 to 20 carbon atoms ( e.g., phenyl, naphthyl), substituted or unsubstituted alkenyl of from 2 to 20 carbon atoms (e.g., vinyl, propenyl),
R₁ can combine R₂ or R₃ to form a substituted or unsubstituted heterocyclic ring of 5 to 8 atoms. This ring contains the nitrogen atom to which R₂ and R₃ are attached in formula (I) and may contain an additional nitrogen atom, or an oxygen or sulfur atom. Examples of such rings include pyridine, quinoline, isoquinoline, thiazole, benzothiazole, thiazoline, oxazole, benzoxazole, imidazole, benzimidazole, and oxazoline.

R₇, R₈, R₉, R₁₀, and R₁₁ are substituted or unsubstituted alkyl of 1 to 20 carbon atoms (e.g., methyl, ethyl, butyl, 2-ethylhexyl, or dodecyl), substituted or unsubstituted aralkyl of from 7 to 20 carbon atoms (e.g., benzyl, phenethyl), substituted or unsubstituted aryl of from 6 to 20 carbon atoms (e.g., phenyl, naphthyl), or substituted or unsubstituted alkenyl of from 2 to 20 carbon atoms (e.g., vinyl, propenyl).

R₈ and R₉, or R₁₀ and R₁₁ can also combine to form a substituted or unsubstituted ring structure of 5 to 8 atoms. The R₈-R₉ ring contains the nitrogen atom to which R₈ and R₉ are attached, and may also contain an additional nitrogen atom, or an oxygen or sulfur atom. The R₁₀-R₁₁ ring may also contain one or more nitrogen atoms, and oxygen atom, a sulfur atom, or any combination thereof. Examples of such rings include pyrrolidine, piperadine, and morpholine.

R₂ or R₃ may each be hydrogen, substituted or unsubstituted alkyl of 1 to 20 carbon atoms (e.g., methyl, ethyl, butyl, 2-ethylhexyl, or dodecyl), substituted or unsubstituted aralkyl of from 7 to 20 carbon atoms (e.g., benzyl, phenthyl), substituted or unsubstituted aryl of from 6 to 20 carbon atoms (e.g., phenyl, naphthyl), or substituted or unsubstituted alkenyl of from 2 to 20 carbon atoms (e.g., vinyl, propenyl). R₂ and R₃ also preferably combine with each other to form a substituted or unsubstituted heterocyclic ring of 5 to 8 atoms. This ring contains the nitrogen atom to which R₂ and R₃ are attached, and may also contain an additional nitrogen atom, or an oxygen or sulfur atom. Examples of such rings include pyrrolidine, piperadine, and morpholine. Either of R₂ or R₃ can combine with R₁ to form a substituted or unsubstituted heterocyclic ring, as described above in reference to R₁.

R₄, R₅, and R₆ are defined the same as described above for R₁, R₂, and R₃, respectively. R₄, R₅, and R₆ may each be the same as or different from R₁, R₂, and R₃.

X^{⊖} represents an anion or an anionic portion of the compound, which forms an intramolecular salt. Any anion that forms a salt compound according to formula (I) that is useful to harden gelatin according to the invention can be used. Preferred anions include a sulfonate ion such as methylsulfonate or p-toluene sulfonate
CF₃SO$\frac{\text{⊖}}{\text{3}}$, BF$\frac{\text{⊖}}{\text{4}}$, PF$\frac{\text{⊖}}{\text{6}}$, and
ClO$\frac{\text{⊖}}{\text{4}}$.

In addition to the above-described alkyl, aralkyl, aryl, alkenyl, and heterocyclic groups, groups, also useful as R₁, R₂, R₃, R₄, R₅, R₆, R₇, and R₈ include substituted alkyl, aralkyl, aryl, alkenyl, and heterocyclic groups. Useful substituents include halogen, alkoxy of from 1 to 20 carbon atoms, aryloxy of from 6 to 20 carbon atoms, a sulfo group, N,N-disubstituted carbamoyl, N,N-disubstituted sulfamoyl, and other groups known to those skilled in the art that do not prevent the compounds from functioning as hardeners according to the invention.

Examples of compounds of formula (I) are shown below in Table I.

The compounds of formula (I) can be made by techniques known to those skilled in the chemical synthesis art. Useful synthesis techniques are described in Journal of the American Chemical Society, 103, 9839 (1981). The preparation of compounds of formula (I) is further described below in the synthesis examples.

The compounds of formula (I) can be used to harden any type of gelatin. Types of gelatin useful in the practice of the present invention include alkali-treated gelatin, acid-treated gelatin, partially phthalated gelatin, double-dipped gelatin (i.e., gelatin treated with both alkali and acid), and the like.

According to the present invention, gelatin is hardened by combining it with a compound of formula (I). The method of hardening gelatin according to the invention can be advantageously be utilized to harden gelatin in photographic layers. The present invention provides rapid hardening of gelatin with little or no after-hardening while avoiding many of the adverse photographic effects found with prior art hardeners, such as speed loss and fog. The hardening compounds of formula (I) also are not highly hygroscopic as are many prior art hardening compounds, making them easy to handle. Additionally, the gelatin hardened according to the invention exhibits desirable physical properties, such as low tackiness.

According to the present invention, gelatin is hardened by combining it with a hardening compound according to formula (I). This is accomplished by techniques known to those skilled in the art. For example, the an aqueous solution of the hardening compound can be applied directly to an unhardened gelatin layer that has been coated on a support. Alternatively, the hardening compound can be mixed with a gelatin-containing coating dispersion shortly before coating it onto a support. Another way of using the compounds of formula (I) is to coat the compound in one layer of a photographic element in a manner such that it will diffuse into other layers of the element to harden those other layers.

The compounds of formula (I) according to the invention can also be used to partially harden gelatin. This is done, for example, by increasing the chain length of the gelatin, as described in U.S. Patent 4,421,847.

The amount of hardener used to harden gelatin according to the present invention will vary according to the purpose for which the gelatin is being used, the degree of hardening desired, and the particular compound of formula (I) that is used. If only a slight amount of hardening is desired, relatively small amounts of hardening compound can be used. If a greater degree of hardening is desired, relatively large amounts of hardener would be used. The amount of hardener used according to the present invention is preferably between 0.01 and 20 weight percent, based on the weight of dry gelatin, and more preferably between 0.05 and 10 weight percent, based on the weight of dry gelatin.

The hardening compound of formula (I) that is used in the present invention can be used alone, in combination with another hardening compound according to formula (I), or in combination with any of a number of hardening compounds or hardening accelerators known in the art. Examples of known hardening compounds include formaldehyde and free dialdehydes, sulfonate esters, epoxides, blocked active olefins, and others, as described in Research Disclosure, item 17643, section X (1978). Examples of known hardening accelerators include nonprotonic solvents, as described in German OLS 2,417,586, tert-amines and their salts, as described in British Patent 1,269,983, and polyhydric alcohols.

The present invention is especially useful for hardening gelatin used in gelatin-containing layers in photographic elements. Such elements are well-known in the art. Examples of elements useful in the practice of the present invention include color negative film, color reversal film, color positive film, color print paper, color reversal print paper, black and white film, black and white paper, X-ray rilm, microfilm, and others well-known in the art. Color films and papers generally contain a red-sensitive silver halide layer, a blue-sensitive silver halide layer, and a green-sensitive silver halide layer. The red-sensitive layer usually has a cyan dye-forming coupler associated therewith, the blue-sensitive layer usually has a yellow dye-forming coupler associated therewith, and the green-sensitive layer usually has a magenta dye-forming coupler associated therewith.

Photographic elements with which the present invention is useful generally include, in addition to the above-described light-sensitive layers, various additional layers, such as filter layers, subbing layers, interlayers, antihalation layers, and the like, as described in Research Disclosure, item 17643 (1978). This Research Disclosure item also describes various addenda, such as surfactants and other coating aids, dye stabilizers, antifoggants, development inhibitor releasing compounds, filter dyes, optical brighteners, antistatic compounds, and the like, that can be included in photographic elements useful in the present invention, either in separate layers or in any of the above-described layers.

The gelatin-containing layers in photographic elements that are advantageously hardened by treatment with the compounds of formula (I) may utilize gelatin as the only binder in the layers, or the gelatin may be combined with other materials. Such materials include, for example, dispersions of water insoluble or slightly soluble polymers, or hydrophilic colloidal polymer materials. Such materials include acrylate polymers, vinyl alcohol polymers, halogenated styrene polymers, poly(sulfonic acid), poly(sulfinic acid), and others described in detail in Research Disclosure, item 17643, section IX (1978).

The invention is further described in the following examples.

### Synthesis Example 1 - Bis(tetramethylformamidinium) ether ditriflate (compound 1)

To a solution of 11.6 g tetramethylurea in 100 ml CH₂Cl₂, 16.8 ml of triflic anhydride in 50 ml CH₂Cl₂ was added dropwise. The mixture was evaporated on a rotatory evaporator at room temperature to yield a yellowish oily residue. The residue was dissolved in 100 ml CH₂Cl₂ and 11.6 g tetramethylurea in 50 ml CH₂Cl₂ was added, at which point a precipitate was formed. The mixture was stirred under nitrogen overnight, after which the precipitate was filtered, washed with CH₂Cl₂, and dried to obtain a colorless crystalline material with a melting point of 258-260°C. IR and NMR analysis indicated that the crystalline material was bis(tetramethylformamidinium) ether ditriflate.

### Synthesis Example 2 - Bis(1-methyl-2-pyridinium)ether ditriflate (compound 2)

To a solution of 0.2 moles of N-methyl-2-pyridone in 150 ml CH₂Cl₂, 16.8 ml of triflic anhydride was added dropwise. A precipitate formed and the mixture was stirred under nitrogen at room temperature for 72 hours. The precipitate was filtered, washed with CH₂Cl₂, and dried to yield a colorless crystalline material with a melting point of 193-195°C. IR and NMR analysis indicated that the material was bis(1-methyl-2-pyridinium) ether ditriflate.

### Comparative Example

A test material was prepared by coating a layer containing a mixture of gelatin at a level of 9.69 g/m² and colloidal silver at a level of 0.48 g/m² onto an Estar^{™} film base. The coated film base was cut into a series of test strips, which were treated with hardening compounds shown in Tables I and II by immersing each strip in an aqueous solution of the compound for 5 minutes, removing the excess solution from the surface of the element, and air-drying at 50°C. The degree of after-hardening was determined by measuring the hardness of the freshly hardened gelatin layer compared to the hardness of a hardened gelatin layer after aging. Hardness of the gelatin layer was measured by gradually immersing the test strip in a 0.8 weight percent aqueous solution of Takamine^{™}, a proteolytic enzyme, at a rate of 0.51 cm/min. The solution was adjusted to a pH of 7.2 and held at 25°C. The wedge length (the length of the strip from where the gelatin was completely removed to the last part of the strip to contact the enzyme solution) was measured and the hardness of the gelatin layer was calculated using the formula:

Compound 21 is compound 8 of U.S. Patent 4,612,280. Compound 22 is compound 1 of EP 162,308. The results of this test are shown in Table III.

Table III shows that compounds 1 and 2 of the invention resulted in no evidence of after-hardening, while compounds 19, 20, and 23 resulted in significant after-hardening. Table III also shows that compounds 1 and 2 of the invention yielded a higher degree of hardening than was achieved by an equivalent molar amount of the hardener compounds 19, 20, 21, 22, or 23.

## Claims

1. A method for hardening gelatin, comprising combining gelatin and a hardening compound,
characterized in that the compound has the formula:
R₁ represents hydrogen, substituted or unsubstituted alkyl of 1 to 20 carbon atoms, substituted or unsubstituted aralkyl of 7 to 20 carbon atoms, substituted or unsubstituted aryl of 6 to 20 carbon atoms, substituted or unsubstituted alkenyl of 2 to 20 carbon atoms, -YR₇, wherein Y represents sulfur or oxygen, and R₇, R₈, R₉, R₁₀, and R₁₁ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms, or R₈ and R₉ together form a substituted or unsubstituted heterocyclic ring, or R₁₀ and R₁₁ are each independently hydrogen or together form a substituted or unsubstituted ring structure, or R₁ together with R₂ or R₃ forms a substituted or unsubstituted heterocyclic ring,
R₂ and R₃ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms, or, taken together with R₁ or each other, forms a substituted or unsubstituted heterocyclic ring,
R₄, R₅, and R₆ are defined as are R₁, R₂, and R₃, respectively, and are the same as or different from R₁, R₂, R₃, and
X^{⊖} represents an anion or an anionic portion of the compound to form an intramolecular salt.

2. A method according to Claim 1 wherein R₁ and R₄ each independently represents hydrogen, substituted or unsubstituted alkyl of 1 to 20 carbon atoms, substituted or unsubstituted aralkyl of 7 to 20 carbon atoms, substituted or unsubstituted aryl of 6 to 20 carbon atoms, substituted or unsubstituted alkenyl of 2 to 20 carbon atoms, -YR₇, wherein Y represents sulfur or oxygen, and R₇, R₈, R₉, R₁₀, and R₁₁ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms, or R₁₀ and R₁₁ are each independently hydrogen, and
R₂, R₃, R₅, and R₆ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms,

3. A method according to Claims 1 or 2 wherein R₁ and R₄ each independently represents hydrogen, substituted or unsubstituted alkyl of 1 to 20 carbon atoms, substituted or unsubstituted aralkyl of 7 to 20 carbon atoms, substituted or unsubstituted aryl of 6 to 20 carbon atoms, substituted or unsubstituted alkenyl of 2 to 20 carbon atoms, -YR₇, or wherein Y represents sulfur or oxygen, and R₇, R₈, and R₉, each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms, and
R₂, R₃, R₅, and R₆ each independently represents substituted or unsubstituted alkyl of 1 to 20 carbon atoms, substituted or unsubstituted aralkyl of 7 to 20 carbon atoms, substituted or unsubstituted aryl of 6 to 20 carbon atoms, or substituted or unsubstituted alkenyl of 2 to 20 carbon atoms.

4. A method according to Claims 1-3 wherein R₁ and R₄ each independently represents

5. A method according to Claims 1-4 wherein at least one combination of two members of R₁, R₂, R₃, R₄, R₅, R₈, R₉, R₁₀, and R₁₁ forms a substituted or unsubstituted ring structure.

6. A method according to Claims 1-5 wherein at least one combination of two members of R₁, R₂, R₃, R₄, R₅, and R₆ forms a substituted or unsubstituted heterocyclic ring.

7. A method according to Claims 1-6 wherein at least one combination of either R₁ and R₂, or R₄ and R₅ forms a substituted or unsubstituted heterocyclic ring.

8. A method according to Claims 6 or 7 wherein the heterocyclic ring is a substituted or unsubstituted pyridylium ring.

9. A method according to Claims 1-8 wherein R₂, R₃, R₅, R₆, R₈, and R₉ each independently represents substituted or unsubstituted alkyl of 1 to 20 carbon atoms.

10. A method according to Claims 1-9 wherein R₂, R₃, R₅, R₆, R₈, and R₉ are each methyl or ethyl.

11. A composition comprising gelatin characterized in that it is hardened by the method of Claims 1-10.

12. A photographic element comprising a support having thereon at least one layer comprising gelatin characterized in that the gelatin is hardened by the method of Claims 1-10.

## Revendications

1. Procédé pour tanner la gélatine dans lequel on combine la gélatine et un composé tannant, composé caractérisé par la formule : où
R₁ représente un atome d'hydrogène, un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone, -YR₇, où Y représente un atome de soufre ou
d'oxygène, et R₇, R₈, R₉, R₁₀ et R₁₁ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, ou un groupe alkényle substitué ou non de 2 à 20 atomes de carbone, ou R₈ et R₉ forment ensemble un hétérocycle substitué ou non, ou R₁₀ et R₁₁ chacun séparément sont un atome d'hydrogène ou forment ensemble une structure cyclique substituée ou non, ou R₁ forme avec R₂ ou R₃ un hétérocycle substitué ou non,
R₂ et R₃ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, ou R₁, R₂ et R₃ pris deux à deux, forment un hétérocycle substitué ou non,
R₄, R₅ et R₆ sont définis respectivement comme R₁, R₂, R₃, et sont identiques ou différents de R₁, R₂, R₃, et
X^{⊖} représente un anion ou une portion anionique du composé qui permet de former un sel intramoléculaire.

2. Procédé selon la revendication 1, dans lequel R₁ et R₄ chacun séparément représente un atome d'hydrogène, un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone, -YR₇, où Y représente un atome de soufre ou d'oxygène, et R₇, R₈, R₉, R₁₀, et R₁₁ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone, ou R₁₀ et R₁₁ sont chacun séparément un atome d'hydrogène, et
R₂, R₃, R₅, et R₆ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone.

3. Procédé selon les revendications 1 ou 2 dans lequel R₁ et R₄ chacun séparément représente un atome d'hydrogène, un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone, -YR₇, ou où Y représente un atome de soufre ou d'oxygène, et R₇, R₈, et R₉ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone, et
R₂, R₃, R₅, et R₆ chacun séparément représente un groupe alkyle substitué ou non de 1 à 20 atomes de carbone, un groupe aralkyle substitué ou non de 7 à 20 atomes de carbone, un groupe aryle substitué ou non de 6 à 20 atomes de carbone, un groupe alkényle substitué ou non de 2 à 20 atomes de carbone.

4. Procédé selon les revendications 1 à 3, dans lequel R₁ et R₄ chacun séparément représente le groupe

5. Procédé selon les revendications 1 à 4, dans lequel au moins une des combinaisons de 2 membres choisis parmi R₁, R₂, R₃, R₄, R₅, R₈, R₉, R₁₀ et R₁₁ forme une structure cyclique substituée ou non.

6. Procédé selon les revendications 1 à 5, dans lequel au moins une combinaison de 2 membres choisis parmi R₁, R₂, R₃, R₄, R₅ et R₆ forme un hétérocycle substitué ou non.

7. Procédé selon les revendications 1 à 6 dans lequel au moins soit R₁ et R₂, soit R₄ et R₅
forment un hétérocycle substitué ou non.

8. Procédé selon les revendications 6 ou 7, dans lequel l'hétérocycle est un cycle pyridylium substitué ou non.

9. Procédé selon les revendications 1 à 8, dans lequel R₂ R₃, R₅, R₆, R₈ et R₉ chacun séparément représente un groupe alkyle substitué ou non de 1 à 20 atomes de carbone.

10. Procédé selon les revendications 1 à 9, dans lequel R₂, R₃, R₅, R₆, R₈ et R₉ sont chacun un groupe méthyle ou éthyle.

11. Composition comprenant de la gélatine caractérisée en ce que la gélatine est tannée par le procédé décrit dans les revendications 1 à 10.

12. Produit photographique comprenant un support portant au moins une couche comprenant de la gélatine caractérisé en ce que la gélatine est tannée par le procédé décrit dans les revendications 1 à 10.

## Patentansprüche

1. Verfahren zur Härtung von Gelatine, bei dem man Gelatine und eine härtende Verbindung zusammenbringt, dadurch gekennzeichnet, daß die Verbindung der Formel entspricht: in der bedeuten:
R₁ Wasserstoff, substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen, substituiertes oder unsubstituiertes Alkenyl mit 2 bis 20 Kohlenstoffatomen, -YR₇, worin bedeuten: Y Schwefel oder Sauerstoff und R₇, R₈, R₉, R₁₀ und R₁₁ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen, oder R₈ und R₉ gemeinsam einen substituierten oder unsubstituierten heterocyclischen Ring, oder R₁₀ und R₁₁ jeweils unabhängig voneinander Wasserstoff oder gemeinsam eine substituierte oder unsubstituierte Ringstruktur, oder R₁ gemeinsam mit R₂ oder R₃ einen substituierten oder unsubstituierten heterocyclischen Ring,
R₂ und R₃ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen, oder gemeinsam mit R₁ oder miteinander einen substituierten oder unsubstituierten heterocyclischen Ring,
R₄, R₅ und R₆ wie R₁, R₂ beziehungsweise R₃ definiert sind und die gleiche oder eine verschiedene Bedeutung wie R₁, R₂ und R₃ haben und
X^{⊖} für ein Anion oder einen anionischen Teil der Verbindung unter Bildung eines intramolekularen Salzes steht.

2. Verfahren nach Anspruch 1, wobei bedeuten: R₁ und R₄ jeweils unabhängig voneinander Wasserstoff, substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen, substituiertes oder unsubstituiertes Alkenyl mit 2 bis 20 Kohlenstoffatomen, -YR₇, worin bedeuten: Y Schwefel oder Sauerstoff und R₇, R₈, R₉, R₁₀ und R₁₁ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen, oder R₁₀ und R₁₁ jeweils unabhängig voneinander Wasserstoff und R₂, R₃, R₅ und R₆ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen.

3. Verfahren nach Ansprüchen 1 oder 2, wobei bedeuten: R₁ und R₄ jeweils unabhängig voneinander Waserstoff, substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen, substituiertes oder unsubstituiertes Alkenyl mit 2 bis 20 Kohlenstoffatomen, -YR₇, oder worin bedeuten: Y Schwefel oder Sauerstoff und R₇, R₈ und R₉ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen und
R₂, R₃, R₅ und R₆ jeweils unabhängig voneinander substituiertes oder unsubstituiertes Alkyl mit 1 bis 20 Kohlenstoffatomen, substituiertes oder unsubstituiertes Aralkyl mit 7 bis 20 Kohlenstoffatomen, substituiertes oder unsubstituiertes Aryl mit 6 bis 20 Kohlenstoffatomen oder substituiertes oder unsubstituiertes Alkenyl mit 2 bis 20 Kohlenstoffatomen.

4. Verfahren nach Ansprüchen 1 bis 3, worin R₁ und R₄ unabhängig voneinander darstellen:

5. Verfahren nach Ansprüchen 1 bis 4, worin mindestens eine Kombination von zwei Gliedern von R₁, R₂, R₃, R₄, R₅, R₈, R₉, R₁₀ und R₁₁ eine substituierte oder unsubstituierte Ringstruktur bilden.

6. Verfahren nach Ansprüchen 1 bis 5, worin mindestens eine Kombination von zwei Gliedern von R₁, R₂, R₃, R₄, R₅ und R₆ einen substituierten oder unsubstituierten heterocyclischen Ring bilden.

7. Verfahren nach Ansprüchen 1 bis 6, worin mindestens eine Kombination von entweder R₁ und R₂ oder R₄ und R₅ einen substituierten oder unsubstituierten heterocyclischen Ring bilden.

8. Verfahren nach Ansprüchen 6 oder 7, worin der heterocyclische Ring ein substituierter oder unsubstituierter Pyridyliumring ist.

9. Verfahren nach Ansprüchen 1 bis 8, worin R₂, R₃, R₅, R₆, R₈ und R₉ jeweils unabhängig voneinander substituiertes oder unsubstituiertes Alkyl mit 1 bis 20 Kohlenstoffatomen darstellen.

10. Verfahren nach Ansprüchen 1 bis 9, worin R₂, R₃, R₅, R₆, R₈ und R₉ jeweils für Methyl oder Ethyl stehen.

11. Zusammensetzung mit Gelatine, dadurch gekennzeichnet, daß sie nach dem Verfahren der Ansprüche 1 bis 10 gehärtet ist.

12. Photographisches Element mit einem Träger, auf dem sich mindestens eine Schicht mit Gelatine befindet, dadurch gekennzeichnet, daß die Gelatine nach der Methode nach den Ansprüchen 1 bis 10 gehärtet ist.
